

## UNITED STATES PATENT OFFICE.

ARTHUR P. HOLLOWAY AND SAMUEL PEACOCK, OF WHEELING, WEST VIRGINIA, AS  
SIGNORS TO WHEELING STEEL CORPORATION, OF WHEELING, WEST VIRGINIA, A  
CORPORATION OF WEST VIRGINIA.

## PROCESS OF PRODUCING SUBSTANTIALLY PURE IRON.

No Drawing.

Application filed June 12, 1924. Serial No. 719,582.

To all whom it may concern:

Be it known that we, ARTHUR P. HOLLOWAY and SAMUEL PEACOCK, both citizens of the United States, residing, respectively, at Wheeling, in the county of Ohio and State of West Virginia, have invented certain new and useful Improvements in Processes of Producing Substantially Pure Iron; and we do hereby declare the following to be a full, clear, and exact description of the invention, such as will enable others skilled in the art to which it appertains to make and use the same.

This invention relates to a process of producing a substantially pure iron product and has for its object to improve the procedures heretofore proposed.

With these and other objects in view the invention consists in the novel steps and combination of steps constituting the process all as will be more fully hereinafter disclosed and particularly pointed out in the claims.

In order that the invention may be the more clearly understood it is said: As is well known, blast furnace pig iron is a crude iron alloy mixture containing say from 60 to 70 per cent free elemental iron and from 30 to 40 per cent of various eutectoids and alloys of iron with carbon, sulphur, phosphorous, silicon and manganese. The well known usual operation of making from such a crude mixture of alloys and iron, a high iron containing product, or one of from, say 99 to 99.9 per cent of iron consists principally in oxidizing out the carbon, sulphur, phosphorus, silicon and manganese present by means of air, and removing the oxidized impurities in the form of molten slags or gaseous reaction products. In the open hearth process, for example iron oxide is also employed, in accordance with the following equation:



But in all such processes the iron is oxidized by the air treatment to an objectionable extent if the metalloids are removed to  $\frac{1}{10}$  per cent, and therefore ferro-alloys are commonly later employed to re-

duce oxides. In the case of employment of ferro-silicon for this reduction the following reaction may take place:



The silica,  $\text{SiO}_2$ , thus produced has a melting point above that of the bath, and can be removed by contact with a base such as an iron or a calcium oxide with either of which it forms a relatively low melting point silicate. But this latter procedure has its disadvantages as will presently appear.

That is, if we consider specifically the open hearth process with which this invention is more directly concerned, its refining process is largely one of the oxidation of the iron by means of air; its controlling factors consist of time, a high temperature and a fluid slag capable of seizing and holding to itself the oxides and impurities present.

The contact between the impurities in the molten and rather crude alloy mixture and the oxidizing reagents is always variable, uncertain and incomplete, so that when one attempts to carry the open hearth process to such an extreme as to cause the elimination of the metalloid impurities down to say below  $\frac{1}{10}$  per cent it is inevitable that a more or less large proportion of the iron is oxidized to such an extent, that there will be present insufficient quantities of metalloid compounds in contact with such oxidized areas to effect a deoxidation of the iron. Thus will be introduced in the iron considerable portions of oxidized metal which must be later deoxidized by a special treatment and it will appear later that this treatment entails objections.

Further, when continuing the contact between the molten metal and the various gases present over a long period of time as is necessary in the prior procedures in order to search out and burn out the diminishing proportions of metalloid impurities with considerable liberation of reaction gases within the metal, as especially is the case when the iron carbide present is converted into elemental iron and carbon monoxide,

a relatively large proportion of gases such as hydrogen, nitrogen, carbon monoxide, etc., are dissolved into or are adsorbed by the molten metal. This latter action is very 5 objectionable, indeed, for it entails undesirable later procedures to get rid of these gases. The presence of such dissolved or occluded gases in the final product is also highly detrimental to the metal when further 10 worked in various industrial procedures. In fact, it may be said that crude pig iron cannot have its total metalloid content reduced below  $\frac{1}{10}$  of one per cent by either the Bessemer or the open hearth process and at the same time escape a highly injurious oxidation and gaseous occlusion in the body of the metal. By the term metalloid above employed, is meant carbon, sulphur, phosphorus and silicon. 15 It is further well known to steel masters, that iron may be heavily oxidized and gassed in removing metalloids, and that by means of a succeeding treatment, in the furnace, ladle, or even in the ingot mold, said iron 20 may be deoxidized by various means. Ferro-alloys are sometimes used for this purpose as illustrated by the following equation:



30 A similar equation illustrates the use of ferro-silicon. But these operations are further well known to never be complete unless an excess of the ferro-alloy is employed, and in such cases, the metalloid silicon may 35 be left in the metal in undesirable proportions and the same may be true of the metal manganese. Accordingly these alloys are employed in restricted proportions.

It is also a fact that no matter how efficient 40 is such ferro-alloy treatment, it does not eliminate the dissolved, the adsorbed nor the occluded gases present.

It is also well known that calcium or 45 aluminum are sometimes added to the molten metal, and that they deoxidize the latter very thoroughly, but they again fail to remove all the occluded or adsorbed gases that may be present. They are further objectionable in their deoxidizing effects as 50 may be illustrated by the following equation:



55 That is, in such cases, there remains in the metal an oxide of the aluminum, or calcium, and these oxides melt only at several hundred degrees above the temperature of the molten iron.

60 It results that as these oxides cannot dissolve, they remain in the metal as disseminated microscopic impurities giving all sorts of trouble later, and especially serving as nuclei for corrosion growths. It is also now 65 believed that the iron-ferrous oxide eutec-

toid which is more commonly known as "burnt iron" is the fundamental cause of perhaps 60 per cent of iron and steel failures in industrial applications, and that this eutectoid depends for its formation on the 70 nascent iron oxide in contact with metallic iron which is inevitably produced in the prior procedures. In other words, it is believed that while the simple admixture of iron and ferrous oxide at very high temperatures forms such eutectoid very slowly, if at all, yet iron at the instant of its oxidation when in contact with an unoxidized iron readily forms such eutectoids at lower temperatures and even at temperatures 80 far below the melting point of either.

The process of this invention, on the other hand, largely avoids the foregoing objections and produces a clean and substantially pure iron product containing less than  $\frac{1}{10}$  per cent 85 of carbon, silicon, sulphur and phosphorous when taken together, and said clean iron product possesses a minimum of dissolved or adsorbed or occluded gases because of the relatively short time of contact with high 90 temperature gases when in the quiescent state. Said clean iron product in addition to the above is not subjected at any stage to a deoxidizing treatment in the cleansing procedure, and hence it is substantially free of 95 oxide disseminations and eutectoids.

The process of this invention therefore, consists simply in working down the silicon, the sulphur and the phosphorus present in the melt by any of the well known open 100 hearth or Bessemer processes for the production of substantially pure iron, but with this important difference; care is taken to not permit the operation to go through the usual decarburizing phase. The molten metal is 105 tapped into a suitable electric furnace, and the temperature is brought up to approximately 1750 degrees C., keeping such metal covered with a suitable low viscosity basic slag, preferably containing from two to six 110 per cent sodium oxide in the form of a sodium silicate admixed with calcium or other silicate. Next, one introduces iron oxide to said bath below said slag in small proportions and only until the molten iron 115 no longer reacts with the iron oxide to produce carbon monoxide. In the meantime the molten metal is kept thoroughly stirred in any suitable manner as for example by the motor action of the electric current employed. The resulting metal having never 120 been oxidized to an objectionable extent as in the prior processes and having never been gassed as in said prior procedures, does not need to be later degassed nor even deoxidized. The electric furnace serves to keep the melt up to the required temperature for metalloids to react while being fractionally treated with iron oxide, but the iron not being at the same time in contact at very 125 130

high temperatures with oxidizing gases as in the prior procedures, there is found to be no need to subject the metal to a deoxidizing, nor to degassing actions in order to produce a substantially pure iron product.

It will now be clear that the process of this invention differs radically from the prior procedures in the following particulars;

The molten bath of crude iron is subjected to a refining process in any suitable and well known fuel fed furnace and in a well known way, but care is taken to so control the air blown into or over the molten mass during the refining as to not produce an objectionable oxidation of the iron. In fact, the refining action in the fuel fed furnace is stopped as soon as the molten mass shows that the iron is practically freed from silicon, and before it is oxidized. No attempt is made in the said fuel fed furnace to decarburize the metal. By this control of the refining action in the furnace, the molten mass is neither oxidized, nor charged with dissolved, occluded or adsorbed gases as heretofore, and consequently no degassing of the final molten product is necessary nor is any deoxidation of the same necessary. In order, however, to get rid of the carbon remaining in the mass, the molten metal is next passed from the fuel fed furnace into an electrically heated furnace, where only sufficient iron oxide is added to the molten bath that is now raised to a high temperature and constantly stirred, to reduce the carbon present as desired.

The iron product thus produced will be found to be slagless and to have an exceptional purity in that the amount of gases contained therein after treatment in the electric furnace will be substantially zero or at most not more than 0.01 per cent. The amount of metalloids can readily be reduced to below 0.10 per cent and ordinarily will not be higher than 0.11 per cent. The amount of other impurities will not exceed .03 per cent, so that the entire product can be easily made to contain 99.85 per cent pure iron.

What is claimed is:—

1. The process of producing an iron product exceeding 99 per cent pure iron, which consists in refining said iron with the aid of air in a suitable fuel fed furnace; stopping said refining action when said iron begins to show signs of decarburization; transferring said iron to an electrically heated furnace; raising the temperature in said last named furnace when out of contact with air to a point higher than is practicable in a fuel-fed furnace sufficiently for any carbon present to reduce any iron oxide present; and agitating the molten mass and feeding iron oxide thereto sufficient for the metalloids present to be reduced to less than 0.15 per cent.

2. The process of producing an iron product exceeding 99.4 per cent pure iron, which consists in refining said iron with the aid of air in a suitable fuel fed furnace, only until said iron begins to show signs of decarburization; cutting off said air and transferring said iron to an electrically heated furnace; raising the temperature of said iron in said electric furnace out of contact with air to a degree sufficient for any carbon present to reduce any iron oxide present; agitating the molten mass; and feeding iron oxide thereto sufficient for the metalloids present to be reduced to less than 0.13 per cent.

3. The process of producing an iron product containing more than 99.5 per cent pure iron which consists in refining in a fuel fed furnace a molten bath of crude iron with the aid of air; shutting off said air when said iron begins to decarburize; transferring the treated iron in its non-oxidized condition to an electric furnace and raising its temperature above 1600° C.; agitating the molten bath thus produced; and feeding iron oxide to said last named bath only in sufficient quantities to react with the impurities present.

4. The process of producing an iron product containing more than 99.7 per cent pure iron which consists in refining in a fuel fed furnace a molten bath of crude iron containing substantially no gases; stopping said refining action before said iron begins to decarburize; transferring the treated iron in its non-oxidized condition to an electric furnace and raising its temperature above 1650° C.; agitating the molten bath thus produced; and feeding iron oxide to said last named bath only in sufficient quantities to react with the carbon and other impurities present.

5. The process of producing an iron product containing more than 99.8 per cent iron, and less than 0.12 per cent of metalloids, which consists in providing a molten bath of iron in a fuel fed furnace; refining said iron until it shows signs of decarburization; stopping said refining action before said iron is decarburized; passing the semi-refined iron into an electrically heated furnace; raising the temperature of said iron in said last named furnace out of contact with air above 1700° C.; agitating the thus heated iron; and gradually adding iron oxide to said iron until its metalloid impurities are reduced below 0.11 per cent.

6. The process of producing an iron product containing more than 99.5 per cent pure iron which consists in refining in a fuel fed furnace a molten bath of crude iron; stopping said refining action before said iron is decarburized; transferring the treated iron in its non-oxidized condition to an electric furnace and raising its temperature above 1700° C.; covering the molten mass with a basic slag to exclude air; agitating the

molten bath in said last named furnace; and feeding iron oxide to said last named bath only in sufficient quantities to react with the impurities present.

7. The process of producing an iron product containing more than 99.8 per cent iron and less than 0.12 per cent of metalloids, which consists in providing a molten bath of iron in a fuel fed furnace; refining said iron in said furnace; stopping said refining action before said iron is oxidized; passing the treated iron into an electrically heated furnace; covering said iron in said last named furnace with a basic slag; raising the temperature of said iron out of contact with air above 1700° C.; agitating the thus heated iron; and gradually adding iron oxide to said iron until its metalloid impurities are reduced below 0.12 per cent.

8. The herein described slagless substantially pure decarburized iron product, the same containing more than 99% iron; less than 0.15% metalloids; and substantially all

of the gases present before decarburization.

9. The herein described slagless substantially pure decarburized iron product, the same containing more than 99.4% iron; less than 0.13% metalloids, substantially all of its gases present before decarburization; and said product being of a character adapted to enhance the corrosion resisting qualities of pure iron.

10. The herein described slagless substantially pure decarburized iron product the same containing more than 99.7% iron; less than 0.11% metalloids; substantially all of the gases that were present prior to its decarburization; and substantially no compounds enhancing the corrosion of the product.

In testimony whereof we affix our signatures.

ARTHUR P. HOLLOWAY.  
SAMUEL PEACOCK.